

## UNITED STATES PATENT OFFICE

2,420,068

## LUBRICANT

Gordon W. Duncan, Westfield, and John C. Zimmer, Union, N. J., assignors to Standard Oil Development Company, a corporation of Delaware

No Drawing. Application January 1, 1944,  
Serial No. 516,704

14 Claims. (Cl. 252—47.5)

1

The present invention relates to mineral lubricating oils, particularly those oils containing additives in the nature of detergents, rust preventives and extreme pressure agents. More particularly, the invention is concerned with compounded mineral lubricating oils which are not subject to or will not show additive separation in the presence of water.

It is known that internal combustion engines, both of the Diesel type and of the spark ignition type, which are subject to long and continuous periods of use as, for example, in long-haul trucking service, high-speed marine service, certain types of aeronautical service, etc., require special lubricating oils commonly designated as heavy duty oils which are compounded especially for this type of service. Mineral lubricating oils which are not so expressly prepared deteriorate relatively rapidly in service, depositing sludge, carbonaceous materials, or varnish-like coatings on such surfaces as cylinder walls, piston skirts, piston ring grooves, etc., and creating an otherwise unclean condition within the engine. For the purpose of counteracting to as great an extent as possible the tendency of mineral lubricating oils to form these deposits, materials of a detergent nature are incorporated into mineral oils destined for heavy duty uses. Generally speaking, these additives are metallic derivatives of organic compounds, but regardless of their exact chemical configuration, they all exhibit the property of reducing or preventing the deposition of carbonaceous or gummy residues and varnish-like films resulting from the deterioration of the lubricating oil. The more common of the detergent additives present in heavy duty oils in amounts ranging from 0.5 to 5% are such compounds as metal naphthenates, metal phenates, metal phenol sulfides, and polysulfides, reaction products of metal phenol sulfides with  $P_2S_5$ , metal carboxylates, metal sulfonates, metal alcoholates, metal salts of esters of acids or thio acids of phosphorus, etc. where the metal ion is a polyvalent metal ion, such as calcium, barium, tin, aluminum, zinc, magnesium, strontium, lithium, nickel, etc. Certain nonmetallic organic compounds are also employed on occasion.

Detergent additives used for improving mineral lubricating oils for heavy duty service are often somewhat hydrophilic and as a result they

2

tend to form emulsions in the presence of water and to drop out of the oil solution, which action results in a heavy duty oil of impaired effectiveness. Normally, mineral lubricating oils used in internal combustion engines are not expected to come in contact with water. However, situations beyond the control of the oil refiner do arise where the prepared lubricating oil does come in contact with water and these occurrences present themselves with sufficient regularity that additive loss through contact with water becomes a serious problem. One instance where loss of additives through contact with water occurs is during shipment of the oil in large size drums or tank cars. Either through atmospheric condensation or leakage of rain water, or because, through oversight, it is left in the drum after cleaning, water is permitted to mix with the oil and precipitate out the detergent additive. Water may also come into contact with the oil in normal automotive operation, particularly during the winter, when low temperatures cause moisture to condense in the crankcase. Another instance where the deleterious action of water on compounded heavy duty oils has been noted is in connection with certain large Diesel installations where, after installation or after the engine has been given a general overhauling, the whole lubricating system including the oil reservoir is washed out with water and then flushed with some of the lubricant intended to be used for normal lubrication. After the flushing operation, the oil is centrifuged to dispose of the water and the oil is then put back into the oil reservoir. If the additive in the oil is hydrophilic in nature, this method of removing water from the oil also removes some of the detergent additive and thus the oil returned to the system is not of the quality desired for such use. It is obvious from the foregoing that some means of retaining detergent additives in the oil even in the presence of water would be very beneficial. The principal object of the present invention resides in the provision of a compounded lubricant for use in the capacity set forth which, when accidentally or otherwise placed in contact or mixed with water, will not lose any substantial amount of the compounding agent. This and other objects to be attained by the use of the present invention will be apparent to those skilled

in the art upon reading the following description.

It has now been discovered that compounded oils having dissolved therein appreciably hydrophilic detergent additives, may be stabilized against emulsification and additive separation by the incorporation of aliphatic amines having from 8-22 carbon atoms to the molecule. Such compounded oils range in viscosity from 90-1000 S. U. S. at 100° F., with pour points usually from -25 to +10° F. and contain from 0.5 to 5% of additives, such as metal phenates, metal phenol sulfides, reaction products of metal phenol sulfonates, metal naphthenates, metal alcoholates, metal salts of the esters of acids or thio acids of phosphorus, etc., or mixtures of the foregoing additives. In general, the metal derivatives of organic compounds utilizable as detergent additives contain ions of polyvalent metals, specific examples of such metals being calcium, barium, aluminum, tin and zinc. The non-metallic detergent additives include materials such as the naturally occurring phosphatides. The usual method of blending compounded oils is to use an oil concentrate of the additive which is dissolved in the mineral oil in the required amount to give the desired product, which solution may be hastened by means of agitation and heat. The detergent additives are frequently made in situ in oil solution so that after removal of the by-products of the reaction, an oil concentrate of the desired additive is obtained directly and this is then used later to make the finished oil by blending it with the proper amount of base stock.

According to the present invention, saturated and unsaturated aliphatic primary amines containing from 8-22 carbon atoms to the molecule will, when present in the compounded heavy duty oil in amounts ranging from 0.005 to 0.5% by weight and preferably 0.01-0.3% by weight, reduce to negligible proportions the emulsification of the oil with water and the additive separation caused thereby. Of the various saturated and unsaturated primary aliphatic amines applicable for the purposes of the present invention, octadecenyl amine (oleyl amine), which is commercially available as a mixture of 50% octadecenyl amine, 25% octadecyl amine and 25% hexadecyl amine, is preferred. Other suitable amines are octadecyl amine (stearyl amine), "Lorol" amine (commercial cocoanut oil amine) and hexadecyl amine.

(cetyl amine). In general, amine derivatives of the fatty acids from animal and vegetable fats are satisfactory for our purpose. The amines may be blended into previously compounded oil by means of heat sufficient to hasten solution. If desired, the amines can be incorporated in the oil concentrates of additives at the time that the concentrates are prepared, in which case the amines will be incorporated in amounts ranging from 1.0 to 20% by weight based upon the weight of the detergent additive present in the oil concentrate, depending upon the concentration of amines desired in the final compounded oil. If desired, the stabilizing agent may be incorporated in concentrates of other additives, such as anti-oxidants bearing corrosion inhibitors, film strength agents, thickeners, pour depressants, and the like. The various detergent additives differ somewhat in their reaction toward water and the amount of detergent additive present is also influential in determining the amount of amines required to effectively reduce additive separation; however, the preferred range of 0.01-0.3% by weight of amines will, in most instances, be found sufficient to give adequate protection against emulsification and additive separation.

A preferred compounded lubricating oil illustrating the present invention is prepared according to the following formula:

|                                                                                                                                                                        | Parts    |
|------------------------------------------------------------------------------------------------------------------------------------------------------------------------|----------|
| Mineral lubricating oil                                                                                                                                                | 100      |
| Mixture of barium tertiary octyl phenol sulfide, calcium sulfonate and the reaction product of barium tertiary octyl phenol sulfide with P <sub>2</sub> S <sub>5</sub> | 0.5-5    |
| Octadecenylamine                                                                                                                                                       | 0.01-0.3 |

For the purpose of demonstrating the effectiveness of aliphatic primary amines as emulsification preventives and stabilizers against additive separation, 50 cc. of an S. A. E. 10 grade mineral lubricating oil containing detergent additives was shaken violently for 20 seconds with 50 cc. of distilled water in a 100 cc. centrifuge tube and then centrifuged for 5 minutes at 1800 R. P. M. In this test, the separation of additive is indicated by a collar of heavy cream-like emulsion lying between the oil and water phases. The volume of the emulsion is an indication of the tendency of the detergent to separate as a result of water contamination and, conversely, of the effectiveness of the stabilizing agent employed.

Table I

| Oil Blend                                                                                                                          | Volume of Emulsion |
|------------------------------------------------------------------------------------------------------------------------------------|--------------------|
| SAE 10 Solvent Extracted Naphthenic Lube Oil                                                                                       |                    |
| 1. +1.5% calcium salt of white oil sulfonic acids.                                                                                 | 8 cc.              |
| 2. (1)+0.5% di-2-ethyl hexylamine.                                                                                                 | 7 cc.              |
| 3. (1)+0.5% di-2-ethyl hexyl amine ethanol.                                                                                        | 3 cc.              |
| 4. (1)+0.3% phenyl ethanol amine (incompletely soluble).                                                                           | 3 cc.              |
| 5. (1)+0.5% diethyl nitrosoamine.                                                                                                  | 3 cc.              |
| 6. (1)+0.5% hepta decyl imidazoline.                                                                                               | 1 cc.              |
| 7. (1)+0.2% hexa decyl amine.                                                                                                      | No emulsion.       |
| 8. (1)+0.3% "Lorol" amine.                                                                                                         | Trace emulsion.    |
| 9. (1)+0.2% octadecyl amine.                                                                                                       | No emulsion.       |
| 10. (1)+0.1% octadecyl amine.                                                                                                      | No emulsion.       |
| 11. (1)+0.05% octadecyl amine.                                                                                                     | No emulsion.       |
| 12. (1)+0.3% octadecenylamine.                                                                                                     | No emulsion.       |
| 13. (1)+0.1% octadecenylamine.                                                                                                     | Do.                |
| 14. (1)+1.0% barium tert. octyl phenol sulfide.                                                                                    | 18 cc.             |
| 15. (14)+0.1% octadecenylamine.                                                                                                    | No emulsion.       |
| 16. Base oil plus 1.75% calcium sulfonate, 1.0% P <sub>2</sub> S <sub>5</sub> treated barium tert. octylphenol sulfide.            | 5 cc.              |
| 17. (16)+0.2% octadecenylamine.                                                                                                    | No emulsion.       |
| 18. Base oil plus 1.5% calcium sulfonate+0.5 % barium tert. octylphenol sulfide+1.0% zinc tert. octylphenol sulfide thiophosphate. | 7 cc.              |
| 19. (18)+0.05% octadecenylamine.                                                                                                   | 3 cc.              |
| 20. (18)+0.1% octadecenylamine.                                                                                                    | No emulsion.       |

The above data clearly show that the agents of this invention, the long chain primary aliphatic amines, are very effective in counteracting additive separation resulting from water contamination of compounded lubricants. It is also shown that other amines, with the exception of heptadecyl imidazoline which is similar in general structure to the long chain primary aliphatic amines, are of little effect in combating this phenomenon.

In a test somewhat similar to the above, 10 cc. of compounded oil is shaken for 20 seconds with 10 cc. of distilled water in a 25 cc. graduated cylinder and allowed to stand one-half hour. The following data illustrate the effectiveness of amines of our preferred class over others:

7. Composition according to claim 1 in which the amine is octadecyl amine.
8. Composition according to claim 1 in which the amine is hexadecyl amine.
9. An improved lubricating oil composition consisting of a mineral lubricating oil containing from 0.5-5% of calcium sulfonate of mineral oil-soluble sulfonic acids and 0.01-0.3% of octadecenyl amine.
10. An improved lubricating oil composition consisting of a mineral lubricating oil containing about 1.5% of calcium sulfonate of petroleum oil-soluble sulfonic acids and 0.1% of octadecenyl amine.
11. An improved lubricating oil composition consisting of a mineral lubricating oil contain-

Table II

| Blend                                                   | Volume of Emulsion               |
|---------------------------------------------------------|----------------------------------|
| <i>SAE 10 Solvent Extracted Naphthenic Lub. Oil</i>     |                                  |
| 1. +1.5% calcium sulfonate.....                         | Oil phase completely emulsified. |
| 2. (1)+0.5% diethylamine ethanol.....                   | Do.                              |
| 3. (1)+0.5% diethylhexylamine.....                      | Do.                              |
| 4. (1)+0.5% s-diphenyl ethylene diamine.....            | 2.5 cc. emulsion.                |
| 5. (1)+0.5% 2,4-utididine.....                          | Oil phase completely emulsified. |
| 6. (1)+0.5% "Lorol" amine.....                          | No emulsion.                     |
| 7. (1)+0.1% "Lorol" amine.....                          | Do.                              |
| 8. (1)+0.5% octadecylamine.....                         | Do.                              |
| 9. (1)+0.1% octadecenylamine.....                       | Do.                              |
| 10. (1)+0.5% octadecenylamine.....                      | 2 cc. emulsion.                  |
| 11. (1)+0.1% octadecenylamine.....                      | 0.5 cc. emulsion.                |
| 12. Baso oil+1.0 barium tert. octyl phenol sulfide..... |                                  |
| 13. (12)+0.5% octadecylamine.....                       |                                  |

In still another test for the water sensitivity of lubricating oil additives, 600 grams of a solvent extracted Mid-Continent S. A. E. 20 lubricating oil containing 1.5% of calcium sulfonate, 0.5% barium tertiary octyl phenol sulfide, and 1.0% of the zinc salt of tertiary octyl phenol sulfide thio phosphate was thoroughly agitated with 1% distilled water in a one liter beaker for one minute. After standing 24 hours, 14 cc. of an emulsion of additive, water, and oil had separated. On repeating the test with the oil containing, in addition, 0.3% of "Lorol" amine, no emulsion or separation of additive was obtained.

What is claimed is:

1. An improved lubricating oil composition consisting of a mineral lubricating oil containing from 0.5 to 5% of an oil-soluble hydrophilic polyvalent metal-containing derivative of an organic compound, said metal compound possessing engine detergent properties, and from 0.01 to 0.3% of an aliphatic primary amine containing from 8 to 22 carbon atoms per molecule.

2. A composition according to claim 1 in which the metal-containing compound is an alkaline earth metal sulfonate.

3. A composition according to claim 1 in which the metal-containing compound is an alkaline earth metal alkylated phenol sulfide.

4. A composition according to claim 1 in which the metal-containing compound is an alkaline earth metal alkylated phenol sulfide reacted with phosphorus sulfide.

5. A composition according to claim 1 in which the metal-containing compound is a mixture of an alkaline earth metal sulfonate and an alkaline earth metal alkylated phenol sulfide reacted with a sulfide of phosphorus.

6. Composition according to claim 1 in which the amine is octadecenyl amine.

35 ing from 0.5-5% of barium tertiary octyl phenol sulfide and 0.01-0.3% of octadecenyl amine.

12. An improved lubricating oil composition consisting of a mineral lubricating oil containing 1% of barium tertiary octyl phenol sulfide and 0.1% of octadecenyl amine.

40 13. An improved lubricating oil composition consisting of a mineral lubricating oil containing about 1.75% calcium petroleum sulfonate, about 1.0% of the reaction product of barium tertiary octylphenol sulfide with  $P_2S_5$ , and 0.2% octadecylamine.

45 14. An improved lubricating oil composition consisting of a mineral lubricating oil containing about 1.5% calcium petroleum sulfonate, 0.5% barium tertiary octylphenol sulfide, about 1.0% zinc tertiary octylphenol sulfide thiophosphate, and about 0.1% octadecylamine.

GORDON W. DUNCAN.  
JOHN C. ZIMMER.

#### REFERENCES CITED

The following references are of record in the file of this patent:

#### UNITED STATES PATENTS

| Number    | Name       | Date          |
|-----------|------------|---------------|
| 2,246,842 | De Groote  | June 24, 1941 |
| 2,270,577 | Bergstrom  | Jan. 20, 1942 |
| 2,280,419 | Wilson     | Apr. 21, 1942 |
| 2,342,099 | Ashley     | Feb. 22, 1944 |
| 2,342,572 | Cook       | Feb. 22, 1944 |
| 2,354,547 | Richardson | July 2E, 1944 |

#### FOREIGN PATENTS

| Number  | Country    | Date          |
|---------|------------|---------------|
| 114,600 | Australian | Feb. 12, 1942 |